

Patented Dec. 22, 1925.

1,566,984

# UNITED STATES PATENT OFFICE.

ROBERT JAY SHOEMAKER, OF CHICAGO, ILLINOIS.

## ELECTROPLATING METHOD AND ELECTROPLATED ARTICLES.

No Drawing.

Application filed October 1, 1923. Serial No. 665,951.

To all whom it may concern:

Be it known that I, ROBERT J. SHOEMAKER, a citizen of the United States, residing at Chicago, in the county of Cook and State of Illinois, have invented certain new and useful Improvements in Electroplating Methods and Electroplated Articles, of which the following is a specification.

My invention relates to methods of electroplating, and more especially to the electroplating of iron or steel articles such, for example, as boiler tubes, sheets, pipes, castings and forgings. The invention is of particular utility in electroplating iron or steel articles with lead inasmuch as it provides, I believe, the only method whereby this operation can be performed with results entirely satisfactory. The invention is of considerable value also in the electrolytic deposition on iron or steel of other metals such as tin, copper and nickel, particularly because affording an expedient for preventing the iron from rusting through the plating with consequent staining of the plating and injury by corrosion to the underlying metal.

Efforts have been made to lead plate by electrolysis iron or steel articles (and hereafter throughout the specification and claims I shall use the term "iron" as covering both species), but so far as I am aware, it has not been found possible heretofore to carry out this operation satisfactorily. If the surface to be covered is slightly greasy or has any scale adhering thereto, even of a microscopic character, the uniformity, density and homogeneity of the lead plating will be affected. It is difficult if not impossible even by pickling the article in acid to clean the surface to be plated sufficiently to make the coating even, non-porous and uniformly adherent. There is also a tendency of the lead to deposit in streaks, that is, in irregular strips with intervening spaces less thickly covered. The reason for this is not fully understood but the phenomenon is recognized by those who have made experiments along this line.

The lead will also deposit more readily and densely on surfaces that are smooth than on rough surfaces so that variations in the character of the iron surface due to inequalities in rolling and other like causes, affect the character of the lead deposited by electrolysis on such surface.

There is also a tendency, during the elec-

trolytic operation, for the lead to "tree out" from the article and eventually produce a short circuit. It does not seem possible to prevent treeing even with mechanical agitation.

Moreover, the lead coating does not adhere to the iron as firmly as is desired. An electro-plated lead boiler tube, for example, if boiled in acids commonly used for testing these articles as to their corrosibility, is likely to blister. Portions of the plating are loosened from the iron so as to be easily rubbed off.

Finally, it has not been found possible, so far as I am aware, to cover an iron with a lead plating produced electrolytically which will be dense enough to prevent corrosion of the iron through the plating. This is also true of iron bodies electro-plated with tin, nickel and copper.

The primary objects of my invention are, therefore: first, to provide a practical method of electro-plating iron articles with lead and, second, an improvement in the methods of electro-plating iron bodies, regardless of the plating metal used, to prevent the rusting through of the iron.

Other less important objects will be referred to in connection with the following description of the preferred manner of practicing the invention.

The method will be described first in connection with lead plating.

(a) The body or article to be plated is first pickled and cleaned in the usual way by sulphuric acid or some other suitable cleansing acid. It may afterward be washed with water but that is not necessary.

(b) It is then immersed in a dilute solution of a copper salt capable of reacting by substitution with the iron, which solution preferably contains an inert agent serving to retard the corrosive action of the solution on the iron. The solution is preferably composed of the following ingredients:

Copper sulphate, 2 parts (by weight); water, 100 parts; glue, 1 part; commercial sulphuric acid, 1 part. Copper chloride may be used in place of copper sulphate. The function of the glue is to slow down the corrosive action of the copper salt solution on the iron. Otherwise the iron would be too deeply bitten by the solution. The glue ingredient, however, need not be used provided care is taken that the articles should

not remain in the bath too long. The reaction is in the sense of the following equations, depending upon whether copper sulphate or copper chloride is used:



This treatment covers the article with a thin coating of copper.

10     (c) The article is then immersed in a weak solution of a mercury salt capable of reacting by substitution with the copper coating. The solution is preferably composed of:

15     Mercuric chloride,  $1\frac{1}{2}$  to 2 ounces; water, 100 pounds; sulphuric acid (commercial), 1 pound.

The acidulation of the solution is optional and in place of mercuric chloride it is possible to use mercuric nitrate, mercuric sulphate or any water soluble salt of mercury.

The reaction is as follows:



25     A film of mercury is formed over the copper coating, the mercury amalgamating with the copper. The effect seems to be to make the copper adhere more firmly to the iron and to fill the pores of the copper coating, which is relatively porous, so that a stratum is provided over the iron base which is very dense, smooth and of uniform character.

Instead of using the solution of mercury salt for producing the mercury film over the copper coating, metallic mercury might be rubbed on the copper coating. The operation, however, is difficult and expensive.

40     (d) Assuming that the article has first been copper coated and then treated with the mercury salt solution, it is then washed to remove the adherent chloride.

45     (e) The next step is the electroplating operation which may be carried on with the use of any suitable electrolyte, such as lead silico-fluoride or, more desirable on account of economy, lead acetate. Using lead acetate, the solution is preferably as follows:

50     Lead acetate, 10 parts (by weight); commercial lime acetate, 10 parts; acetic acid, 1 part; water, 100 parts.

The electrolyte is kept in slow agitation by means of a pump or compressed air during the process. The function of the lime acetate, in place of which ammonium acetate

55     or sodium acetate may be used, is primarily to reduce internal resistance. Incidentally the organic impurity, to-wit, compounds of pyroligneous acid, serve to prevent treeing. The current flow should be approximately one ampere per square foot of surface plated and the potential from four to six volts. Metallic lead is used as a positive pole.

60     It will be understood that in the electroplating of articles with metals other than lead, the preparation of the article for treat-

ment in the electrolytic cell would be the same as described in steps (a) and (d).

65     The operation of copper coating described as step (b) may be used to advantage without subsequent step (c) in a copper electroplating operation precedent to immersion of the article in the electrolytic cell. In this case the solution should be strengthened to contain about 10% copper salt.

70     Steps (b) and (c), whereby the body is covered with a coating consisting of an amalgam of copper and mercury, may be advantageously used in preparing billets for cold drawing into pipes, tubes, and the like. The coating provides an excellent metallic lubricant which, if necessary, may be removed by pickling in case it is necessary to anneal the billet between draws.

75     The operations described as steps (c) and (d) might be used advantageously as a pre-treatment in the lead tin or nickel plating of copper, brass or bronze articles.

I claim:

1. Improvement in the method of electroplating iron articles which consists in covering the surface of the article to be plated with a permanently adherent film of mercury and a metal with which mercury will amalgamate and thereafter electro-plating said surface.

2. Improvement in the method of electroplating iron articles which consists in coating the surface of the article to be plated with copper and covering the coppered surface with a film of mercury prior to the electro-plating operation.

3. Method of electro-plating iron articles which consists in immersing the article in a solution of a copper salt capable of reacting by substitution with the iron to coat the article with copper, covering the coppered surface with a film of mercury, and then electro-plating the mercury covered surface.

4. Method of electro-plating iron articles which consists in immersing the article in a solution of a copper salt capable of reacting by substitution with the iron to coat the same with copper, immersing the article in a solution of a mercury salt capable of reacting with the copper to produce an amalgamation of metallic mercury with the copper coating, and then electro-plating the surface so treated.

5. Method of electro-plating iron articles which consists in immersing the article in a solution of a copper salt capable of reacting by substitution with the iron and containing an agent for retarding the corrosive action of the solution on the iron to coat the article with copper, covering the coppered surface with a film of mercury, and then electro-plating the mercury covered surface.

6. Method of electro-plating iron articles which consists in immersing the article in a

solution of copper salt capable of reacting by substitution with the iron and containing an agent for retarding the corrosive action of the solution on the iron to coat the article 5 with copper, immersing the article in a solution of a mercury salt capable of reacting by substitution with the copper to produce an amalgam of metallic mercury with the copper coating, and then electro-plating the 10 surface so treated.

7. Method of electro-plating an iron article which consists in immersing the article in an acidulated solution of copper sulphate or its equivalent to produce a reaction in 15 the sense of the equation



immersing the article in a solution of mercuric chloride or its equivalent to produce 20 a reaction in the sense of the equation



and then electro-plating the article.

8. Method of electro-plating an iron article which consists in immersing the article 25 in an acidulated solution of copper sulphate or its equivalent, and containing glue, to produce a reaction in the sense of the equation



immersing the article in a solution of mercuric chloride or its equivalent to produce 35 a retarded reaction in the sense of the equation



and then electro-plating the article.

9. Improvement in the method of electro-plating iron articles with lead which 40 consists in coating the surface of the article to be plated with copper and covering the coppered surface with a film of mercury prior to the electro-plating operation.

45 10. Method of electro-plating iron articles with lead which consists in immersing the article in a solution of a copper salt capable of reacting by substitution with the iron to coat the article with copper, covering the coppered surface with a film of mercury, and then electro-plating the mercury covered surface.

50 11. Method of electro-plating iron articles with lead which consists in immersing the article in a solution of a copper salt capable of reacting by substitution with the iron to coat the same with copper, immersing the article in a solution of a mercury salt capable of reacting with the copper to produce an amalgamation of metallic mercury with the copper coating, and then electro-plating the surface so treated.

55 12. Method of electro-plating iron articles with lead which consists in immersing the article in a solution of a copper salt

capable of reacting by substitution with the iron and containing an agent for retarding the corrosive action of the solution on the iron to coat the article with copper, covering the coppered surface with a film of 70 mercury, and then electro-plating the mercury covered surface.

13. Method of electro-plating iron articles with lead which consists in immersing the article in a solution of copper salt capable of reacting by substitution with the iron and containing an agent for retarding the corrosive action of the solution on the iron to coat the article with copper, immersing the article in a solution of a mercury salt 75 capable of reacting by substitution with the copper to produce an amalgam of metallic mercury with the copper coating, and then electro-plating the surface so treated.

14. Method of electro-plating an iron article with lead which consists in immersing the article in an acidulated solution of copper sulphate or its equivalent immersing the article in a solution of mercuric chloride or its equivalent and then electro-plating the 80 article.

15. Method of electro-plating an iron article with lead, which consists in immersing the article in an acidulated solution of copper sulphate or its equivalent, and containing 85 glue, immersing the article in a solution of mercuric chloride or its equivalent and then electro-plating the article.

16. Method of producing a metal coating on iron articles which comprises treating 100 the article with a solution of copper salt capable of reacting by substitution with the iron and containing a retarding agent to slow the corrosive action of the copper salt solution on the iron.

17. Method of producing a metallic coating on iron articles which comprises treating the article with a solution of copper sulphate or its equivalent containing glue to retard the corrosive action of the solution 110 on the iron.

18. Method of producing a metallic coating on iron articles which comprises first covering the article with a coating of copper and then covering the copper surface with 115 mercury.

19. Method of producing a metallic coating on iron articles which comprises treating the article with a solution of a copper salt capable of reacting by substitution with the iron and then treating the coppered surface with a solution of a mercury salt capable of a substitution reaction with the copper coating.

20. Method of producing a metallic coating on iron articles which comprises treating the article with a solution of a copper salt capable of reacting by substitution with the iron and containing an agent to retard the corrosive action of the copper salt solution

on the iron, and then treating the coppered surface with a solution of a mercury salt capable of a substitution reaction with the copper coating.

5 21. Improvement in the method of electroplating which consists in covering the surface to be electroplated with a copper coating and covering the copper coating with a film of mercury.

10 22. Method of electroplating which comprises dissolving in the electrolyte a soluble acetate of an alkali or alkaline earth together with pyroligneous acid to prevent treeing.

15 23. An electroplated iron article having between the iron surface and the electroplat-

ing a stratum of mercury amalgamated with copper.

24. An electroplated iron article having between the iron surface and the electroplat- 20 ing first a coat of copper in contact with the iron and over the copper a film of mercury.

25. A lead plated iron article having between the surface of the iron and the lead plating first a copper coating and over the 25 copper coating in contact with the iron a film of mercury.

26. An electroplated metal body having under the electroplating a coating of copper and over the copper a film of mercury.

ROBERT JAY SHOEMAKER.